

June 2, 1931.

K. D. ROBINSON

1,807,875

METHOD OF ELECTROPLATING AND PRODUCT THEREOF

Filed Oct. 21, 1926

Fig. 1



Fig. 2



Fig. 3



INVENTOR

Karl D. Robinson

BY

Philip George Richter

ATTORNEYS

## UNITED STATES PATENT OFFICE

KARL DAVIS ROBINSON, OF NEW YORK, N. Y., ASSIGNOR TO THE MERIDEN GRAVURE COMPANY, OF MERIDEN, CONNECTICUT, A CORPORATION OF CONNECTICUT

## METHOD OF ELECTROPLATING AND PRODUCT THEREOF

Application filed October 21, 1926. Serial No. 143,303.

This invention relates particularly to an improved method of electroplating upon a metal cathode which before electroplating has received a coating of a permeable substance, and more specifically to an improved method of causing the adherence of this colloid coating to the metal, and to the product of this improved method.

The especial object of the present invention is to produce an intimate and firm adherence of the coating to the metal on which it is coated, and to produce a deposit of metal the texture of which can be controlled by the nature of the coating and its handling during the electroplating process.

A further object of the invention is to produce specifically a metal printing plate having firmly united thereto a printing surface consisting essentially of a colloid or like permeable substance.

In certain classes of printing plates, as for instance in collotype, it has been usual to coat a glass plate with a substratum consisting of gelatin and sodium silicate, and then coating the gelatin emulsion forming the printing surface of the plate on this substratum, the substratum adhering to the glass plate because of the common silicate content and the colloid adhering to the substratum because of the common gelatin content. This collotype printing, however, is usually effected at comparatively low speeds and a colloid thus coated on glass is satisfactory at low speeds. When, however, a permeable coating is applied to a metal plate, such as aluminum or zinc, and the plate is operated at high speed, the colloid coating tends to strip from the metal plate during the printing operation, and this is liable to occur even at low speed.

By the present invention, a substratum is produced containing in an intimate admixture a permeable substance as a colloid and a material similar to the plate, so that the colloid adheres to the metal plate in like manner as does the colloid adhere to the substratum used with a glass plate, so that these metal plates can be used at very high speed without the colloid stripping.

A preferred embodiment of the invention will now be described as employed in the pro-

duction of a printing plate. It will be understood, however, that the method is applicable for producing objects other than printing plates and therefore is not to be limited to the production of this specific article, but is applicable to electroplating on a wide range of metal cathodes.

The production of a printing plate, however, will be described as illustrative only of the invention, both as to the method and product features, in which the metal plate or cathode is aluminum, the colloid is gelatin, and the electroplating metal is zinc.

In the accompanying drawing, Figures 1, 2 and 3 illustrate symbolically the various steps of the process, Figure 1 showing the metal plate with a colloid coating; Figure 2 the coated plate and the electrolytically deposited metal, and Figure 3 the product of Figure 2 with the addition of a printing emulsion.

Broadly considered, the method consists in utilizing the plate as the cathode and depositing upon the cathode prior to the electroplating step a thin film of a permeable material, that is, a colloid or colloidal material permeable to the metal ion of the electrolyte, such as gelatin or other suitable colloid, which is allowed to set to the gel condition before immersion of the cathode in the electroplating bath; immersing the cathode to cause the colloid to swell to the desired condition with respect to permeability; and then passing for a suitable time, depending upon the amount of metal it is desired to deposit, an electric current of required amperage until this desired thickness of the metal is obtained.

As a specific example of carrying out the invention in accordance with the best practice now known to me, the cathode is in the form of an aluminum plate, which is cleaned, rinsed, dipped into a mild alkali, such as sodium carbonate solution, and then dipped in a suitable hydrochloric acid solution, this preparation of the plate being customary for preparing an aluminum plate for electroplating.

The aluminum plate thus prepared is then coated, preferably by whirling, with a solu-

tion of a suitable colloid, such as gelatin, containing preferably sufficient hydrochloric acid or other suitable acid to bring the solution into a suitable condition with respect to 5 acidity as compared with the acidity of the electrolyte, so that there will be no undesired change in the physical and chemical characteristics of the gelatin when introduced into the electrolyte. That is to say, it is preferred that the pH of the gelatin solution be 10 so adjusted to the pH of the electrolyte that degree of swelling and other characteristics of the gelatin reach an equilibrium quickly when the gelatin is introduced into the electrolyte. The whirling of the plate is continued until the gelatin coating is dried. The electroplating bath in the preferred embodiment of the invention is slightly acid and a satisfactory bath is one of zinc sulphate, ammonium chloride and sodium acetate in suitable proportions. The colloid coated plate is immersed in the bath, which is maintained preferably at a temperature not exceeding 20° C. until the gelatin has swollen sufficiently 25 to have the desired permeability, ten minutes usually being sufficient for this. An electric current of suitable amperage is then passed between the cathode plate and the anode of zinc; and the plate may be gently 30 rubbed or swabbed during the electroplating, which obliterates such hydrogen bubbles as penetrate the gelatin surface and will insure an even disposition of the metal. After a sufficient amount of zinc has been deposited 35 on the aluminum plate, the plate is removed from the bath and then rinsed and dried, preferably by whirling, and if any deposits of zinc have penetrated through the face of the gelatin layer, these deposits, which are 40 but lightly attached to deposited metal lying below the face of the gelatin layer, can be removed, without injury to the gelatin layer, by gentle buffing while the plate is whirling after the gelatin has become dried.

45 This method of electroplating produces a deposit of zinc on the aluminum plate, the metallic zinc being deposited between the interstices of the permeable gelatin and becoming intimately admixed or interlaced with 50 the gelatin coating. By this is meant that metal is deposited upon those areas of the metal plate to which the metal ion of the electrolyte has access, the metal not being deposited upon such areas of the plate as are 55 protected from the metal ion by the substance of the permeable membrane.

If the gelatin layer is sufficiently thick to 60 avoid any outcropping of zinc, and if this gelatin layer is otherwise suitable for printing purposes, the plate thus formed may serve directly as a printing plate.

In the best practice of the invention, however, I prefer to coat the plate initially with 65 a thickness of gelatin sufficient for the purpose of providing the zinc-gelatin substratum

and, after the substratum has dried, coating the plate with a colloid emulsion or coating especially prepared for printing purposes, this printing coating being applied to the prepared plate, preferably by whirling. Adhesion of this second printing coating to the substratum is effected by means of the common gelatin content, the gelatin of the printing coating adhering to the gelatin of the substratum, and the substratum adhering to the metal plate by reason of the metal in the substratum. This results in the production of a plate from which the printing coating will not strip even when the plate is used at high printing speeds. 70 75 80

It may be stated that by a suitable choice of the colloid and its condition as to swelling, and by controlling the evolution of hydrogen at the cathode, which may be done by regulating the composition of electrolyte, current density or other suitable means, a wide control of the texture of the surface of the plate is possible. By proper control of the hydrogen, there will be a fine network of hydrogen bubbles formed at the surface of the metal plate, and these cause a building up of small cylinders of metal spaced in relationship to the bubbles. When this coating is dried, as above stated, and the excess metal above the surface removed by light buffing, a 90 95 100 velvety mat surface can be obtained; and by proper control of the hydrogen any surface from the maximum smoothness to a rough matte can be obtained.

If desired, the gelatin substratum may be removed by hot water or other suitable means, and an electroplated product obtained having a deposit of zinc on the aluminum of a maximum smoothness or of a matte surface, which is desirable in the production of certain articles. 105

It will, of course, be understood that the coating used for the production of printing plates will have the characteristics which will enable the finished plate to be used for high speed printing such as ability to receive and transfer ink at high printing speeds. 110

While the invention has been described as particularly adapted for producing printing plates, it will be obvious that other metals both for the plate and for the metallic deposit, and other electroplating baths can be employed without departing from the invention, and that permeable membranes other than gelatin may be used depending upon the products it is desired to produce, and that the invention may be employed in the production of other products than printing plates, and the invention is therefore not to be limited to the specific details hereinbefore described. 115 120 125

What I claim is:

1. The method of electroplating on metal articles which consists in coating the metal 130

with a permeable colloid prior to the electro-plating step, drying the coating, causing the colloid to swell to the required condition of permeability, then plating on the article a metal through the colloid in an electrolytic bath.

5 2. The method of electroplating on metal articles which consists in coating the metal with gelatin prior to the electroplating step, 10 drying the gelatin, causing the gelatin to swell to the required condition of permeability, and then plating on the article a metal through the gelatin in an electrolytic bath.

15 3. The method of electroplating on metal articles which consists in coating the metal with gelatin prior to the electroplating step, drying the gelatin, causing the gelatin to swell to the required condition of permeability, then plating on the articles a metal 20 through the gelatin in an electrolytic bath, and drying the gelatin coating.

25 4. The method of producing a printing plate which consists in coating a metal plate with a permeable colloid, drying the colloid, causing the colloid to swell to the required condition of permeability, subjecting the plate and coating to an electrolytic bath containing a metallic salt, which deposits on the plate in metallic form between the interstices of the colloid, drying the applied coating, and applying a printing surface over the dried coating.

30 5. A printing plate having a permeable colloid coating secured thereto by electro-plating with a metal through the interstices of the colloid which forms part of the finished plate.

35 6. A printing plate having a permeable colloid coating secured thereto by electro-plating with a metal through the interstices of the colloid, and a colloid printing surface coated over the first colloid coating.

40 7. A printing plate having a gelatin coating secured thereto by electroplating with a metal through the interstices of the gelatin, and a printing surface coated over the gelatin.

45 8. An aluminum printing plate having a gelatin coating secured thereto by electroplating with zinc through the interstices of the gelatin.

50 55 the gelatin.

9. An aluminum printing plate having a gelatin coating secured thereto by electroplating with zinc through the interstices of the gelatin to form a substratum, and a gelatin printing surface applied over the substratum.

In testimony whereof, I have hereunto set my hand.

KARL DAVIS ROBINSON.